

G. W. BERNAUER.  
STIFFENING MATERIAL FOR SHOES.  
APPLICATION FILED NOV. 8, 1920.

1,426,538.

Patented Aug. 22, 1922.

Fig. 1.



Fig. 2.



George W. Bernauer,  
Inventor.  
by Small & Small  
His Attorneys.

# UNITED STATES PATENT OFFICE.

GEORGE W. BERNAUER, OF ST. CHARLES, MISSOURI.

## STIFFENING MATERIAL FOR SHOES.

1,426,538.

Specification of Letters Patent. Patented Aug. 22, 1922.

Application filed November 8, 1920. Serial No. 422,448.

To all whom it may concern:

Be it known that I, GEORGE W. BERNAUER, a citizen of the United States, residing at St. Charles, in the county of St. Charles, State of Missouri, have invented a certain new and useful Stiffening Material for Shoes, of which the following is a specification.

This invention has for its prime object 10 the provision of a blank to be placed beneath the fore part of the vamp of a shoe prior to the "pulling over" operation and impregnated with a stiffening composition which is softened by the application of moderate 15 heat so as to render the blank pliable and thus enable said operation and the subsequent lasting operation to be performed without difficulty.

A further object is the provision of a 20 blank having substantially the same strength as leather, thereby affording support for the tip of the vamp during the "pulling over" and lasting operations.

A further object is the provision of a 25 blank impregnated with a composition which is entirely unaffected by climatic conditions or the temperature of the foot during wear of the shoe, is thoroughly water proof, will not stick to the last and will retain the 30 original shape of the toe under hardest usage.

In the accompanying drawing Figure 1 is a plan view of the blank showing its 35 skived edges, and Figure 2 is a longitudinal section of an unlasted upper showing the toe-cap, vamp and linings and the preferred location of the blank with respect to these elements.

In carrying out the invention I combine 40 about two pounds of rosin with one-quarter pound of dry shellac and heat for approximately one hour at 400 to 500 degrees Fahrenheit, then allowing to cool to about 212 degrees. When the latter temperature is 45 reached there is added about one pound of glue, one-quarter pound of dry white lead and one-half ounce of carbolic acid, the mixture being stirred to intimately combine the several ingredients and the heat maintained 50 substantially at the point last mentioned.

Preferably the glue is first softened by standing several hours in alcohol or other solvent diluted with a small quantity of water and is mixed with the lead before addition to the composition as above described, and if it is desired to produce flexi-

ble blanks suitable for the finer grades of dress shoes the composition is rendered less stiff by the addition of approximately one-half pint of a softener made of pulverized 60 rosin dissolved in alcohol and then heated to about 212 degrees Fahrenheit. Obviously, if a smaller quantity of the softener is used, very stiff blanks, adapted for heavy boots and shoes, will be produced.

While the addition of the carbolic acid is not essential it is very useful in that it stops the foaming which ensues on addition of glue and lead and causes the glue to harden quickly after the composition has been 70 applied to the material of which the blank is formed. Preferably the material employed is medium weight flannelette or cotton flannel which is soft and absorbent and this is run through or immersed in the composition while the latter is hot and then allowed to dry on suitable racks.

The blank A depicted in Figure 1 is cut from the stiffened material by suitable dies and its margin B reduced by skiving or 80 scouring after which it is inserted between the inner and outer linings C—D beneath the fore part of the vamp E upon which the toe-cap F is stitched at G.

The parts in the flattened condition shown 85 in Figure 2 are first subjected to approximately 200 degrees (Fahrenheit) of dry heat from an electric or gas heater so as to soften the blank for the "pulling over" operation and thereafter placed, on the last, within a 90 toe-steaming machine where the hot vapor serves to soften the leather as well as the blank so that the lasting operation, which follows immediately, may be performed 95 without difficulty.

Having thus fully described the invention, what I claim as new and desire to secure by Letters-Patent is:—

1. A stiffener for parts of shoes consisting of a suitably shaped blank of absorbent material impregnated with a stiffening composition, comprising rosin, glue and white lead, which renders said blank substantially inflexible when dry and softens upon application of a degree of heat insufficient to injure the leather of the shoe.

2. A stiffener for parts of shoes consisting of a suitably shaped blank of absorbent material impregnated with a stiffening composition, comprising rosin, shellac, glue and white 110 lead, which renders said blank substantially inflexible when dry and softens upon appli-

cation of a degree of heat insufficient to injure the leather of the shoe.

3. A stiffener for parts of shoes consisting of a suitably shaped blank of absorbent material impregnated with a stiffening composition, comprising rosin, shellac, glue, phenol and white lead, which renders said blank substantially inflexible when dry and softens upon application of a degree of heat 10 insufficient to injure the leather of the shoe.

4. A stiffener for parts of shoes consisting of a suitably shaped blank of absorbent material impregnated with a stiffening composition, comprising shellac, glue and white 15 lead, which renders said blank substantially

inflexible when dry and softens upon application of a degree of heat insufficient to injure the leather of the shoe.

5. A stiffener for parts of shoes consisting of a suitably shaped blank of absorbent 20 material impregnated with a stiffening composition, comprising shellac, glue, phenol and white lead, which renders said blank substantially inflexible when dry and softens upon application of a degree of heat insuf- 25 ficient to injure the leather of the shoe.

GEORGE W. BERNAUER.

Witnesses:

RALPH KOHLENHARFF,  
FRANK LEHMANN.